

2,724,687

## BATHS FOR THE DEPOSIT OF GOLD ALLOYS BY ELECTROPLATING

Victor Spreter and Jean Mermilliod, Geneva, Switzerland

 No Drawing. Application July 21, 1952,  
Serial No. 300,127

Claims priority, application Switzerland May 8, 1952

6 Claims. (Cl. 204—43)

Baths for electrogilding, irrespective of the gold alloy colour which they serve to obtain, have almost identical compositions. Indeed, gold, copper, silver, nickel, cadmium or zinc are contained therein as soluble cyanides, that is to say alkaline metal-cyanides. In addition these baths contain, according to case, phosphates, sulphites, carbonates and free cyanides, these salts being intended for improving either the electric conductivity or the penetrating power of the bath, or the brilliance of the deposits obtained.

When such a bath has just been prepared, it is found that, for a given temperature and current density, its yield (considered from the point of view of the metal deposited, as compared to the current consumed), through being lower than 100%, is the highest found in the above mentioned operating conditions. Indeed whether the bath is used or not, it is found that the yield compared to the current consumed regularly falls with time and may go down to nearly 10% after a certain number of days: the bath is said to have aged.

The consequences of such ageing are disastrous: when thick gilding is involved (over 1 or 2 microns), the necessary duration for obtaining such gilding considerably increases as time passes and finally becomes unacceptable; if light gilding is involved (colour setting), the ageing state of the bath is one more variable which must be reckoned with in the already ticklish bath working in order to keep constant the colour of the deposited alloy.

The present invention relates to a bath for the deposition of gold alloys by electroplating, which is not subject to ageing, that is to say, the yield of which, computed on the basis of the current consumed as compared to the weight of the metal deposited, measured when the bath has just been prepared, remains constant during the whole life of the bath.

This bath, as those already known, contains the gold intended for plating in the form of alkaline aurocyanide. It is characterized by the fact that, apart from the said aurocyanide, it is free from any other cyanide and by the fact that it contains an organo-metallic compound of the metal to be alloyed with gold, soluble in water and having a low dissociation constant.

It is this organo-metallic compound, other than a cyanide, which supplies the metal to be alloyed with the gold at the time of formation of the gold alloy deposit. The metal of this compound may thus be copper, nickel, cadmium, zinc. It has been found that when the metal to be alloyed with gold is introduced into the bath in a form other than cyanide, the bath does not age.

The said organo-metallic compound may include in its molecule the group  $-\text{N}(\text{CH}_2\text{COO})_2$ . It may be a salt of an organic acid and of the metal to be alloyed with gold, insofar as this salt has a low dissociation constant. Among the salts fulfilling this condition, one may mention those of the acids presenting in their molecule the above mentioned group, such as those of imido-diacetic acid and its derivatives, for instance ethylene-diamino-

tetraacetic acid, nitrilo-triacetic acid, anthranilic-diacetic acid, uranil-diacetic acid, aminomalonic-diacetic acid.

On the other hand, conducting salts such as phosphates and sulphites can be completely omitted from the bath and replaced by the potassium and sodium salts of the organo-metallic compound above referred to. The bath does not contain any free cyanide.

Baths in accordance with the present invention and the organo-metallic compound of which is a salt of ethylene-diamino-tetraacetic acid, are remarkable for their following properties:

They do not age, that is to say that their yield, computed on the basis of the current consumed under given electrolysis conditions, remains constant during their whole life;

They give brilliant gold alloy deposits, the assay of which may be adjusted by changing the electrolysis factors; They make it possible to obtain a very quick increase of the thickness of the deposits (ten times more quickly than with the baths used hitherto). A current density of 2 to 3 amperes per sq. decimeter (18.5 to 28 amperes per sq. foot) at the cathode gives excellent deposits;

Their penetrating power into the cavities of the object placed at the cathode far exceeds that of ordinary cyanide baths;

They remain extremely limpid during use;

Their content of copper salt (being the one most generally present in these baths) may be adjusted very easily by colorimetry owing to the blue tint of said salt.

The following examples give the composition of baths, in conformity with the present invention, and the manner of using them:

### EXAMPLE 1

*Bath for the deposition of thick coatings (pink colour)*  
g. per litre

|                                                          |     |
|----------------------------------------------------------|-----|
| Gold (as potassium aurocyanide)                          | 12  |
| Cu (as copper salt of ethylene-diamino-tetraacetic acid) | 2.5 |
| Zn (as zinc salt of ethylene-diamino-tetraacetic acid)   | 2   |
| Ni (as nickel salt of ethylene-diamino-tetraacetic acid) | 2   |
| Potassium salt of ethylene-diamino-tetraacetic acid      | 5   |

The pH of the bath is adjusted to approximately 8 by adding either ethylene-diamino-tetraacetic acid or potassium carbonate.

By using this bath at a temperature of 60° C., with a stainless steel anode and under a current density of 2.5 amperes per sq. decimeter (23.2 amperes per sq. foot) of cathode, very brilliant gold alloy deposits are obtained, assaying approximately 19 carats. The thickness of the deposit is about 25 microns per hour (1/1000 inch per hour), which corresponds approximately to a 35% yield for the current consumed.

### EXAMPLE 2

*Bath for the deposition of thin gold coatings (yellow and pale yellow colours)*  
g. per litre

|                                                          |   |
|----------------------------------------------------------|---|
| Gold (as potassium aurocyanide)                          | 1 |
| Ni (as nickel salt of ethylene-diamino-tetraacetic acid) | 2 |
| Potassium salt of ethylene-diamino-tetraacetic acid      | 5 |

By using this bath at a temperature of 60° C. with a stainless steel anode, one may, when adjusting the cathode current density between 0.3 and 0.8 amp. per sq. decimeter (2.8 and 7.5 amp. per sq. foot), obtain any gold tint, from the 24 carats yellow to very pale yellow, and all intermediate tints in-between. This bath has an

absolutely remarkable penetrating power and stability; maintaining the colour of the deposit from one operation to another is very easy.

## EXAMPLE 3

*Bath for the deposition of thin gold coatings (green colour)*

|                                                | g. per litre |
|------------------------------------------------|--------------|
| Gold (as potassium aurocyanide)                | 1            |
| Cd (as cadmium salt of nitrilo-triacetic acid) | 2            |
| Potassium salt of nitrilo-triacetic acid       | 5            |

By using this bath at a temperature of 60° C. with a stainless steel anode, one may, by adjusting the cathode current density between 0.3 and 0.5 amp. per sq. decimeter (2.8 and 4.65 amp. per sq. foot), obtain all the tints of green colour gold.

## What we claim is:

1. A bath for the deposition of an alloy of gold with at least one metal selected from the group consisting of copper, nickel, cadmium and zinc, said bath containing exclusively an alkaline aurocyanide and at least one organometallic compound selected from the group consisting of the copper, nickel, cadmium and zinc salts of ethylene-diamino-tetraacetic acid, nitrilo-triacetic acid, anthranilic-diacetic acid, uranyl-diacetic acid and amino-malonic-diacetic acid, whereby the yield, computed on

the basis of the current consumed as compared to the weight of metal deposited, remains constant during the whole life of the bath.

2. A bath according to claim 1, in which the said organo-metallic compound is a salt of ethylene-diamino-tetraacetic acid.

3. A bath according to claim 1, in which the said organo-metallic compound is a salt of nitrilo-triacetic acid.

4. A bath according to claim 1, in which the said organo-metallic compound is a salt of anthranilic-diacetic acid.

5. A bath according to claim 1, in which the said organo-metallic compound is a salt of uranyl-diacetic acid.

6. A bath according to claim 1, in which the said organo-metallic compound is a salt of aminomalonic-diacetic acid.

## References Cited in the file of this patent

## UNITED STATES PATENTS

2,660,554 Ostrow Nov. 24, 1953

## OTHER REFERENCES

Thews: Metal Finishing, September 1951, page 83.